

# UNITED STATES PATENT OFFICE.

WILFRED VAN WART, FRANZ WILLIAM POPP, AND JOSEPH JOHN BRADLEY,  
OF BIRMINGHAM, ENGLAND.

## ALLOY.

SPECIFICATION forming part of Letters Patent No. 633,743, dated September 26, 1899.

Application filed December 23, 1897. Serial No. 663,228. (No specimens.)

To all whom it may concern:

Be it known that we, WILFRED VAN WART, FRANZ WILLIAM POPP, and JOSEPH JOHN BRADLEY, subjects of the Queen of Great Britain, residing at Birmingham, England, have invented certain new and useful Improvements in Alloys, (for which we have obtained patents in Great Britain, No. 12,287, bearing date June 5, 1896, and No. 19,640, bearing date 10 September 5, 1896,) of which the following is a specification.

Our invention has for its main object the production of a new or improved alloy having for its base or major portion aluminium, and which improved metal shall comprise among other advantages extreme lightness, strength, durability, and non-corrosiveness, whereby it is especially adapted for the manufacture of tubes of all kinds, sheets, wire, 15 castings, and the like and for other industrial uses.

By the employment of our improved alloy we are enabled to greatly improve upon the good qualities claimed for aluminium and add 20 a very considerable number of others which aluminium does not possess.

As is well known, aluminium by itself, though valuable for some purposes, is practically useless for the majority of industrial 25 trades in which metals are used, as it is very unreliable when being worked up, and therefore will not produce satisfactorily such articles as tubes, sheets, wire, castings, and the like. Moreover, castings made of it cannot 30 be successfully used by reason of its extreme softness. For a similar reason aluminium affords comparatively little tensile strength, but is weak under compression and bending tests.

Now in order to overcome these difficulties and to provide for the object that we have in view we proceed as follows: In or about the following proportions we take of aluminium, say, one hundred parts; of copper, from one 40 to ten parts; of zinc, from one-eighth of a part to six parts; of silver, from one-eighth of a part to six parts; of tin, from one-eighth of a part to four parts; of phosphorus, say, from one-sixteenth of a part to one part. These 45 several ingredients are all well mixed together in the following or other suitable manner, which can be somewhat varied, according to

requirements: The copper is first of all melted. The zinc is then added by gradual additions after warming same. At the same time 55 the silver is added, so that the stirring or working may proceed evenly upon the whole of these ingredients during the process of mixing. Aluminium is then added. The pot is now withdrawn, and the tin is added, together 60 with phosphorus. The admixture of ingredients is then well stirred until the whole has become well melted and amalgamated, so as to produce a homogeneous compound metal before pouring. The introduction and use of 65 phosphorus we find by experiments imparts solidity to the mass of metal and at the same time improves the elasticity or ductility.

Our metal will be found especially valuable for the manufacture of the tubes forming the 70 framing and for the rims of the wheels and for other of the component parts of cycles, autocars, and other road-vehicles, and which, while retaining all the advantages of aluminium or of aluminium and its alloys as generally understood, will be without many of the 75 disadvantages appertaining to the latter. By varying the quantity of the ingredients within the proportions named the metal may be made harder or softer, according to requirements.

It will be understood from the formula above set forth for purposes of example that where fractional parts are given they are based upon their relation to the other parts. For instance, one-eighth of a part to four parts equals, say, one-eighth of a pound to four 85 pounds, and so on.

Having now described our invention, what we claim as new, and desire to secure by Letters Patent, is—

The herein-described improved alloyed metal consisting of aluminium, copper, zinc, tin, silver and phosphorus, the percentage of aluminium therein being from ninety per 95 cent. upward substantially as specified.

In witness whereof we have hereunto set our hands in presence of two witnesses.

WILFRED VAN WART.  
FRANZ WILLIAM POPP.  
JOSEPH JOHN BRADLEY.

Witnesses:

EDWD. BAETON PAYNE,  
CHARLES JOHN LUCAS.